

April 23, 1974

C. E. SHOEMAKER

3,806,356

FLUX AND METHOD OF COATING FERROUS ARTICLE

Filed Aug. 9, 1972



3,806,356  
**FLUX AND METHOD OF COATING FERROUS  
ARTICLE**

Carlyle E. Shoemaker, Bethlehem, Pa., assignor to  
Bethlehem Steel Corporation, Bethlehem, Pa.  
Filed Aug. 9, 1972, Ser. No. 275,610

Int. Cl. C23c 1/08; C23f 17/00

U.S. CL. 117—50

11 Claims

## ABSTRACT OF THE DISCLOSURE

This invention relates to the process of coating ferrous articles by the molten metal immersion method, more particularly to the provision of an aqueous flux applied to said article prior to the metal coating thereof. Specifically, the process includes cleaning the ferrous article, wetting the surfaces with an aqueous flux of fluosilicic acid, with up to four compounds from the group consisting of hydrochloric acid, hydrofluoric acid, potassium fluoride and zinc chloride, drying said flux on the surface, immersing said article in a molten metal bath consisting essentially of at least 25% by weight aluminum, balance essentially zinc, and after removal from the bath, shaking off excess metal and cooling to yield a ferrous article having a continuous and adherent layer of said aluminum-zinc alloy.

## BACKGROUND OF THE INVENTION

This invention is directed to the concept of coating ferrous metal articles, by the hot metal immersion method, to enhance the article's appearance and resistance to corrosion attack. To effect such results, an adherent and continuous layer of a corrosion resistant material on the ferrous article is essential. The prior art using various combinations of salts and acid has met with limited success in galvanizing and aluminizing processes due to production costs, processing controls and product performance.

Typically, the ferrous article to be coated had to be cleaned of grease and scale (oxides of iron) prior to the application of the metallic coating. In a continuous strand operation, i.e. strip or wire, the material preferably is cleaned and then bathed in an oxide reducing atmosphere, and without exposing it to the atmosphere is immediately immersed in a molten metal bath containing the coating metal. For batch operations, particularly for large structural members, atmospheric exclusion is virtually impossible. Accordingly, alternatives for protecting the cleaned surfaces were found. Generally, the procedure was to apply a thin flux coating following the cleaning, and then immersing the flux coated ferrous article into the molten metal bath. Naturally, the nature of the fluxing composition is important to its effect on the ferrous base, for its ability to provide a proper surface for the reception of a metal coating, which is both continuous and adherent. Thus there is a relationship between the flux and coating metal.

While the prior art has made some significant contributions in the area of galvanizing and aluminizing, such efforts have not been totally satisfactory for preparing ferrous surfaces for the reception of an aluminum-zinc coating. However, with the discovery of a fluosilicic acid containing flux, an effective means was found to prepare the surface of a ferrous article for subsequent coating by an aluminum-zinc alloy.

## SUMMARY OF THE INVENTION

This invention relates to the process of coating ferrous articles by the molten metal immersion method, more particularly to the provision of a suitable aqueous flux containing fluosilicic acid for applying to the surfaces of the ferrous article prior to the metal coating thereon. In its preferred embodiment, said process includes cleaning the ferrous surfaces to remove grease, etc., pickling to remove scale, dipping directly into a flux bath containing from about 2 to about 15% by weight,  $H_2SiF_6$ , with up to about a total of 25%, by weight of the flux bath, of the compounds from the group consisting of HCl, HF, KF, and  $ZnCl_2$ , where the quantity of said compounds depends on the alloy content of the ferrous article, drying the flux in situ, and immersing the flux coated ferrous article in a molten metal bath of at least 25% by weight aluminum, balance essentially zinc. Upon withdrawal from the molten bath, and removal of excess metal, such as by bumping, the metallic coating solidifies to produce a ferrous article having a continuous, adherent coating of an aluminum-zinc alloy.

## BRIEF DESCRIPTION OF THE DRAWING

The figure is a flow sheet illustrating the preferred sequence of steps followed in carrying out the process of this invention.

## DETAILED DESCRIPTION OF THE PREFERRED EMBODIMENT

Turning now to a more detailed review of the invention, as set forth in the illustrated flow sheet of the figure, it will be seen that the present invention provides an improved hot metal immersion coating procedure yielding a ferrous article having a continuous, adherent coating of an aluminum-zinc alloy thereon.

The coating method generally comprising wetting the cleaned scale free ferrous article with an aqueous solution containing from about 2 to 15%, by weight,  $H_2SiF_6$ , with up to a total of about 25%, by weight, of the compounds selected from the group consisting of HCl, HF, KF, and  $ZnCl_2$ . Following the wetting thereof, the ferrous article is dried such as by heating to a low temperature of up to about 400° F. to remove all signs of dampness. This is important, especially from a safety standpoint, to avoid splashing of the subsequently applied molten coating metal.

The dry flux coated ferrous article is then immersed for from 2 to about 5 minutes, depending on the depth of metallic coating desired, in a molten metal bath containing at least 25%, by weight, aluminum, preferably up to about 70%, balance essentially zinc. After removal, excess coating metal is removed, such as bumping or agitating the coated ferrous article, where it may be cooled by air or water quenching. The resulting product exhibits a continuous, adherent alloy coating on the processed ferrous article.

At this juncture, it should be made clear that as used herein, the term "article" is intended to include strip and wire (treated in a continuous manner), and shapes, such as structural members treated in a batch process. Actually, the greatest benefits from this invention are realized in the batch treatment of ferrous shapes, such as large structural steel members used in the construction industry. Though not limiting, the further description and exemplary showings shall be directed to batch operations.

Optimum results, particularly in the treatment of alloy structural steels, were observed with fluxing compositions containing from about 4.0 to 8.0%, by weight,  $H_2SiF_6$ ,

and about 5.0 to 20.0%, by weight, of a plurality of the remaining compounds listed above. For example, from the standpoint of coating coverage, adherence and appearance, a preferred fluxing composition is as follows:

| Compound:  | Percent by weight | 5  |
|------------|-------------------|----|
| $H_2SiF_6$ | 5.5               |    |
| HF         | 3.5               |    |
| KF         | 9.0               |    |
| $ZnCl_2$   | 1.8               |    |
| Water      | Balance           | 10 |

To further illustrate the effectiveness of the fluxing composition on surface coverage, evaluations were made on two common grades of structural steel, with variations in flux composition. The said variations are listed in Table I, 15 with the results in Table II.

TABLE I

| Components: | Flux baths, weight percent |     |     |     |     |    |    |     |     |     |     |     |     |    |    |
|-------------|----------------------------|-----|-----|-----|-----|----|----|-----|-----|-----|-----|-----|-----|----|----|
|             | A                          | B   | C   | D   | E   | F  | G  | H   | J   | K   | L   | M   | N   | P  | Q  |
| $H_2SiF_6$  | 10                         | 10  | 10  | 10  | 10  | 10 | 10 | 10  | 5   | 5   | 5   | 2.5 | 5   | 5  | 5  |
| HCl         |                            |     |     |     |     |    |    |     |     | 5   |     |     |     |    |    |
| HF          | 3.5                        | 1.8 | 1.8 | 1.8 | 3.5 | 5  | 5  | 1.8 | 1.8 | 1.8 | 3.5 | 0.9 | 3.5 | 5  | 5  |
| KF          | 10                         | 10  | 10  | 10  | 10  | 10 | 10 | 10  | 10  | 10  | 10  | 5   | 10  | 10 | 10 |
| $ZnCl_2$    | 2                          | 2   | 2   | 2   | 2   | 2  | 2  | 2   | 2   | 2   | 2   | 1   | 2   | 2  | 2  |

TABLE II

| Steel: | Percent surface covered, 5 minutes dip |     |       |     |     |       |     |     |     |     |     |     |     |     |     |
|--------|----------------------------------------|-----|-------|-----|-----|-------|-----|-----|-----|-----|-----|-----|-----|-----|-----|
|        | A                                      | B   | C     | D   | E   | F     | G   | H   | J   | K   | L   | M   | N   | P   | Q   |
| A372   | 100                                    | 100 | 99    | 100 | 95  | 98    | 97  | 100 | 100 | 100 | 100 | 100 | 100 | 100 | 100 |
| A36    | 99                                     | 100 | ----- | 99  | 100 | ----- | 100 | 100 | 100 | 100 | 100 | 100 | 100 | 100 | 100 |

While it may be gleaned from the foregoing tabulation, as it pertains to alloyed steels, optimum results or surface coverage were noted with the richer fluxes, i.e. those containing a plurality of said compounds. However, with leaner ferrous articles, such as mild or low carbon steels, simpler flux combinations, with the components named, may be formulated.

For instance, aqueous fluosilicic acid may be used alone or in combination with only one or two of the remaining components. Some combinations which have been found suitable for mild carbon steel sheet and strip are listed below.

TABLE III

| Components: | Flux baths, weight percent |       |     |
|-------------|----------------------------|-------|-----|
|             | N                          | P     | Q   |
| $H_2SiF_6$  | 10                         | 10    | 10  |
| HCl         |                            |       | 8.7 |
| KF          | 10                         | ----- | 2   |
| $ZnCl_2$    |                            |       |     |

Since the foregoing represents the preferred embodiments of this invention, it is contemplated that variations may be effected herein by those skilled in the art, particularly after reading these specifications. Accordingly, no limitation is intended to be imposed on this invention except as set forth in the appended claims.

I claim:

1. A method of forming a continuous alloy coating consisting of from 25% to about 70%, by weight aluminum, balance essentially zinc, on a ferrous article, comprising the steps of cleaning said ferrous article to remove grease and oxides from the surfaces thereof to be 70 coated, immersing said article in an aqueous acidic flux

consisting essentially of fluosilicic acid, and up to four compounds from the group consisting of hydrochloric acid hydrofluoric acid, potassium fluoride and zinc chloride, removing said article from the aqueous acidic flux, drying said article by heating to a low temperature, and immersing the article in a molten bath containing said aluminum-zinc coating alloy.

2. The method claimed in claim 1 wherein the fluosilicic acid is present in amount between about 2 to 15%, by weight, of said aqueous flux.

3. The method claimed in claim 2 wherein at least one of said four compounds is present up to a total amount of 25%, by weight, of said aqueous flux.

4. The method claimed in claim 2 wherein said fluosilicic acid is present in an amount between about 4 to 8%.

5. The method claimed in claim 4 wherein at least one

of said four compounds is present in an amount between about 5 to 20%, by weight, of said aqueous flux.

6. The method claimed in claim 5 wherein a plurality of said four compounds are present in said aqueous flux.

7. The method claimed in claim 5 wherein at least three of said four compounds are present in said aqueous flux.

8. A flux for the treatment of a ferrous article prior to its immersion in a molten bath containing an aluminum-zinc alloy, comprising an aqueous acidic solution consisting essentially of from 2 to 15%, by weight, of fluosilicic acid, and a total of from 5 to 20%, by weight, of at least one compound selected from the group consisting of hydrochloric acid, hydrofluoric acid, potassium fluoride, and zinc chloride.

9. The flux claimed in claim 8 wherein said fluosilicic acid is present in an amount between about 4 to 8%.

10. The flux claimed in claim 9 wherein a plurality of said four compounds are present in the aqueous flux.

11. The flux claimed in claim 10 wherein at least three of said four compounds are present in the aqueous flux.

## References Cited

## UNITED STATES PATENTS

- 60 2,671,737 3/1954 Jominy et al. ----- 117—51  
2,907,104 10/1959 Brown et al. ----- 117—49  
2,174,551 10/1939 Cinamon et al. ----- 117—52

## FOREIGN PATENTS

- 65 1,025,603 4/1966 Great Britain ----- 117—52

RALPH S. KENDALL, Primary Examiner

M. W. BALL, Assistant Examiner

U.S. Cl. X.R.

117—50, 114 C, 114 A; 148—23